

Feb 13, 1940

R. P. KOEHRING

2,190,237

METHOD OF MAKING A COMPOSITE METAL STRUCTURE

Filed Dec. 30, 1937



INVENTOR  
Roland P. Koehring  
BY  
Spencer Hardman & Felt  
his ATTORNEYS

## UNITED STATES PATENT OFFICE

2,190,237

## METHOD OF MAKING A COMPOSITE METAL STRUCTURE

Roland P. Koehring, Dayton, Ohio, assignor to  
General Motors Corporation, Detroit, Mich.,  
a corporation of Delaware

Application December 30, 1937, Serial No. 182,411

7 Claims. (Cl. 75—22)

The present invention relates to metallic structures and more particularly to a method of fabricating porous metal structures that have a metallic ingredient dispersed within the interstitial pores thereof.

It is an object of the present invention to provide a method of fabricating a porous alloy structure from a porous metal matrix which comprises, impregnating a previously fluxed porous metal matrix with a metal at such a temperature and for such a time as to prevent the impregnating metal from dissolving the porous metal matrix, and then subsequently heating the impregnated matrix and thereby causing at least a part of the impregnating metal to substantially uniformly diffuse into the metal of the matrix and form an alloy therewith without destroying the continuity of the porous metal matrix.

It is a further object, in some cases, to impregnate the porous metal matrix with a mixture of two metals, one of which is readily alloyable with the metal of the matrix and the other of which is not readily alloyable with the metal of the matrix, the impregnated matrix being subsequently heated to cause the readily alloyable metal to uniformly diffuse into the metal of the matrix and alloy therewith without destroying the continuity of the matrix and leave the less readily alloyable metal dispersed within the pores of the matrix.

Further objects and advantages of the present invention will be apparent from the following description, reference being had to the accompanying drawing wherein a preferred embodiment of the present invention is clearly shown.

In the drawing:

The single figure is a diagrammatic view, illustrating a method of applying loose uncompacted metal powder in a layer upon a strong metal back and sintering the loose layer in situ upon the metal back to form a porous metal matrix directly bonded to the back by an alloy bond.

The present invention is directed to a low temperature impregnating method whereby readily alloyable metals may be impregnated into a metal matrix or sponge at low temperatures and subsequently the impregnated sponge may be heated to cause uniform alloying of all or a part of the alloyable impregnating metal with the sponge without any harmful effects, such as destroying the continuity of the sponge.

In practicing such a method it is possible to substantially uniformly impregnate a copper sponge with pure tin and later heat the im-

regnated sponge and thereby cause the tin substantially uniformly diffuse into the copper of the matrix and alloy therewith to form bronze sponge in situ, having substantially the same continuous structure as the original copper sponge. Likewise, a pure copper sponge may be impregnated with a mixture of lead and tin. The impregnated sponge may be subsequently heated to cause the tin to uniformly dissolve in the copper to form an alloy therewith leaving the less alloyable lead uniformly dispersed within the pores of the newly formed bronze sponge.

The present method can be advantageous carried out with any number of metallic sponge for example, copper, iron, nickel, bronze sponge copper-nickel sponges etc., together with sponges which include a non-metallic disperse material therein, such as graphite. Impregnating metals such as tin, silver, aluminum, bismuth, bismuth-lead alloys, tin-lead alloys, tin-silver alloys and many other metals and alloys thereof can all be used to advantage.

While the following description is directed to impregnating and subsequently alloying or partially alloying the impregnated metal with sponge or matrix which is directly bonded to steel back, it should be understood that the method is not limited in this respect and may be used with equal success on sponges that have no supporting backs.

Referring to the drawing a loose layer 10 of the desired thickness of the finely divided matrix forming metal powder is applied onto a relatively strong metal strip 11, such as steel, as the strip 11 moves along under the hopper 12 at a suitable slow uniform speed. The loose matrix-forming metal powder 13 in hopper 12 runs out by the aid of gravity upon strip 11 and is preferably smoothed thereon by a suitable adjustable smoothing device 14 to provide a smooth-surfaced uniform layer 10 of loose metal powder upon the strip 11.

The moving metal strip 11 with the loose layer 10 thereon passes into the sintering chamber 2 and is there heated in a non-oxidizing or reducing atmosphere to such a temperature and for such a time as will cause the loose or only slightly compacted metal particles to molecularly bond together and form a strong highly porous matrix lining 15 and at the same time to molecularly bond to the metal strip 11. During this sintering process the thickness of the loose powder layer 10 is materially reduced due to shrinkage so that the porous metal lining 15 emerging at 2 from the sintering chamber 20 is about one-

less than the loose powder layer 10 which is chamber 20. Hence, the original thickness of the powder layer 10 is made such as will the desired thickness and density of the sintered porous metal matrix lining 15. This can easily be determined by trial for any given ingredients in the matrix-forming metal powder 13. Strip 11 is of steel it is preferably, but not necessarily, first copper plated before the loose powder layer 10 is applied thereon since it has been found that the sintered porous lining 15 will bond somewhat more strongly to a copper surface than it will to a steel surface. However, the porous matrix lining 15 will bond successfully to uncoated clean steel surface. The temperature of the sintering chamber is accurately controlled by suitable means and is preferably heating electric heating elements 25.

The highly porous matrix lining 15 preferably comes from the sintering chamber 20 into the outer jacketed cooling chamber 22 where it is held under non-oxidizing or reducing conditions to substantially prevent oxidation of the porous metal matrix. The reducing or non-oxidizing gas is admitted to the sintering chamber through an inlet 23 and then escapes through an outlet 24 of the cooling chamber 22. In this manner the non-oxidizing atmosphere is sent in both chambers 20 and 22 and at a pressure slightly in excess of atmospheric pressure to assure that no atmospheric gases enter the aforementioned chambers.

The density or porosity of porous matrix lining can be accurately controlled, if desired, by suitably sizing the lining by a pressure operation, for example, by passing strip 11 with the porous lining 15 bonded thereto between pressure plates 30 and 31 illustrated in the drawing. These plates 30 and 31 may be set any desired distance apart so as to compress the lining 15 to any desired thickness, thereby reducing the porosity thereof.

After the porous metal lining 15 has been bonded to strip 11 the lined strip is preferably cut into short lengths which may then be immersed in a fluxing bath either under vacuum or under atmospheric conditions, or the strip may be painted with the fluxing material, such as ammonium or zinc chloride, rosin and alcohol, borax, etc., or exposed to an atmosphere of a gassing gas. The fluxed strip is then immersed in a molten bath of the desired impregnating metal. It is preferable to utilize a vacuum during

impregnation to draw the occluded air and gases from the pores of the matrix prior to immersing the same in the impregnating metal bath and then apply pressure to the bath by increasing the pressure thereover to force the impregnating metal into the pores of the immersed metal sponge. The impregnated metal sponge is then removed from the impregnating bath and preferably cooled, although the cooling step is not necessary to the success of the steps that follow. Subsequently the sponge may be heated under non-oxidizing or reducing conditions to a temperature well above the impregnating temperature, to cause the impregnated metal to alloy or partially alloy with the metal of the matrix. In trying out the aforementioned steps it has been discovered that the fluxing step may be eliminated if the sintered metal matrix is impregnated before exposure to atmospheric air since the surfaces therein are substantially free from oxidation or other surface films.

A specific example of the fabrication of a copper

sponge impregnated with tin by such procedure is as follows: Uncompacted copper powder on a steel strip is preferably sintered at a temperature of approximately 1900° F. for from 10 to 15 minutes, which causes the copper particles to sinter together to form a strong sponge having a continuous metallic network which is alloyed by an alloy bond to the supporting back. This copper sponge is then fluxed by immersion in ammonium chloride solution or any other suitable flux disclosed herein and is subsequently immersed in a bath of molten tin which is preferably maintained at a temperature of approximately 450° to 500° F., the melting point of tin being 449.4° F. Prior to the immersion of the sponge in the impregnating bath the aforementioned vacuum is applied and then under evacuated conditions the sponge is immersed and pressure applied for a period of immersion approximately from 1 to 2 minutes, which is sufficient to cause complete and uniform impregnation of the tin into the sponge. The tin impregnated copper sponge, if desired, may next be cooled to set the impregnated metal although this step is not necessary. The impregnated sponge is then heated under non-oxidizing or reducing conditions to a temperature well above 500° F., for example 1000° to 1900° F. for a period up to 10 minutes. During this heating period the tin, which readily dissolves copper, at these higher temperatures uniformly diffuses into the copper matrix thereby forming a uniform and homogeneous bronze without destroying the continuity of the matrix. The period of heating, the temperature of the heating step, or both, may be varied to accomplish partial alloying of the tin.

In a like manner a tin-lead mixture can be used as the impregnating alloy for a copper matrix in which instance the impregnating bath is maintained up to fifty degrees above the melting point of the tin-lead alloy. In this case, the subsequent heating of the impregnated sponge, which has a uniform dispersion of the lead alloy therethrough, causes the tin to diffuse into the copper matrix and leave the lead, which is not readily alloyable with either copper or bronze, in a finely divided state within the pores of the bronze matrix.

In a similar manner a bronze sponge can be utilized in which case, as the tin diffuses therein, the tin content of the bronze, is changed to a higher percentage than was present in the original sponge.

In place of tin such aforementioned metals as bismuth, cadmium, bismuth-lead or silver-tin etc. can be used as impregnating metals for copper or bronze sponges, in each case the impregnating temperature being just above the melting point of the impregnating metal or alloy and the subsequent heating step being slightly below the melting point of the porous metal sponge when a pure metal sponge is used, and preferably below the melting point of the highest melting constituent metal when an alloy sponge is used. Likewise, iron sponge can be readily impregnated and subsequently alloyed with aluminum and similarly nickel sponge can be transformed into Monel sponge by impregnating with copper etc.

The present method is decidedly advantageous when it is desired to impregnate and subsequently alloy a sponge with a readily alloyable metal since such a method as herein described prevents any substantial dissolving action by the impregnating metal on the sponge whereby the structure of the sponge in its final form is substantially

similar to the structure of the sponge prior to the impregnating and alloying steps.

While the embodiment of the present invention as herein disclosed, constitutes a preferred form, it is to be understood that other forms might be adopted, all coming within the scope of the claims which follow.

What is claimed is as follows:

1. The steps in the method of making a metallic structure comprising: providing a porous metal matrix of copper which has intercommunicating voids therein by sintering together finely divided non-compacted copper powder, fluxing said matrix with a suitable flux so that the flux penetrates within the intercommunicating voids of the matrix, immersing the fluxed matrix in a molten bath of tin at a temperature only slightly above the melting point of tin and for such a short period of time that the tin while flowing within the intercommunicating voids of the matrix has no substantial dissolving action upon the metallic structure of the matrix, removing the impregnated matrix from the bath, and then heating the impregnated copper matrix to a temperature well above the melting point of tin whereby the tin diffuses into the copper and simultaneously progressively raises the melting point of the alloy formed by the copper and the tin and thereby prevents the continuity of the resultant matrix from being destroyed to form a bronze matrix with intercommunicating voids therein.
2. The steps in the method of making a porous metal structure having a metal held within the pores thereof comprising: providing a porous metal matrix having intercommunicating voids therein by sintering together finely divided non-compacted metal powder, fluxing said matrix with a suitable flux so that the flux penetrates within the intercommunicating voids of the matrix, impregnating the matrix with the mixture of metals, one of which readily alloys with the metal of the matrix and the other of which does not readily alloy with the metal of the matrix by immersing the porous metal matrix in a molten bath of an alloy of the two impregnating metals which bath is maintained at a temperature slightly above the melting point of said alloy for a short time only and thereby preventing any substantial dissolving action by the readily alloying impregnating metal upon the matrix, then subsequently heating the impregnated metal matrix to a temperature sufficiently high to cause the readily alloyable metal to uniformly diffuse into the matrix to form an alloy therewith, and leave the remainder of the impregnating metal dispersed within the pores of the metal matrix, and then cooling the alloyed matrix.
3. The steps in the method of making a porous bronze structure having lead dispersed in the pores thereof comprising: providing a copper matrix having intercommunicating voids therein by sintering together finely divided non-compacted copper powder, fluxing said matrix with a suitable flux so that the flux penetrates within the interstitial pores of the matrix, impregnating the copper matrix with lead and tin by immersing the copper matrix in a molten bath of lead and tin for a short time only, which bath is maintained at a temperature only slightly above the melting point of the lead-tin alloy then subsequently heating the impregnated metal matrix to a temperature well above the melting point of the lead-tin alloy and thereby causing the tin

to uniformly diffuse into the copper matrix and form a bronze therewith without destroying the continuous structure of the matrix, and leaving the lead dispersed within the interstitial pores of the bronze matrix.

4. The steps in the method of making a metallic structure comprising: providing a porous metal matrix of homogeneous character by sintering together finely divided non-compacted metal powder, fluxing said matrix with a suitable flux so that the flux penetrates the interstitial pores of the matrix, impregnating the fluxed porous metal matrix with a mixture of metals which includes one metal that is readily alloyable with the metal in the matrix and another metal which is not readily alloyable with the metal of the matrix, at a temperature only slightly above the melting point of the impregnating alloy and for such a time as to prevent any substantial dissolving action by the readily alloyable metal upon the matrix, then subsequently heating the impregnated porous metal matrix at a temperature well above the impregnating temperature and thereby causing the readily alloyable metal to diffuse into the matrix and form an alloy therewith without destroying the continuous structure of the matrix and leaving the less alloyable metal dispersed within the pores of the matrix.

5. The steps in the method of making a composite metal structure comprising: uniformly distributing a loose layer of uncompacted metal powder upon a relatively strong non-porous metal supporting back, subjecting the loose layer in situ upon said back, to such a temperature and for such a time as will cause the loose metal particles to molecularly bond together and form a relatively highly porous matrix having intercommunicating voids therein and simultaneously cause said matrix to molecularly bond to said metal back, impregnating the porous metal matrix with a metal which is readily alloyable with the metal of the matrix at a temperature only slightly above the melting point of the impregnating metal and for such a time as to prevent the impregnating metal from having substantial dissolving effect on said matrix, and then subsequently heating the impregnated metal matrix to a temperature sufficiently high to cause substantially uniform diffusion of at least a portion of the impregnating metal into the porous metal matrix and thereby form an alloy in situ with the matrix without destroying the continuity of the matrix.

6. The steps in the method of making a composite metal structure comprising: uniformly distributing a loose layer of uncompacted metal powder upon a relatively strong non-porous supporting back, subjecting the loose layer, in situ upon said back, to such a temperature and for such a time as will cause the loose metal particles to molecularly bond together and form a relatively highly porous matrix having intercommunicating voids therein and simultaneously cause said matrix to molecularly bond to said metal back, impregnating the porous metal matrix with a mixture of metals one of which readily alloys with the metal of the matrix and the other of which does not readily alloy with the metal of the matrix at a temperature slightly above the melting point of the metal mixture and for such a time as to prevent any substantial dissolving action by the readily alloyable impregnating metal upon the matrix, then subsequently heating the impregnating metal matrix to a tem

erature sufficiently high to cause at least a portion of the readily alloyable metal to uniformly diffuse into the matrix to form an alloy therewith, and leave the remainder of the impregnated metal dispersed within the pores of the metal matrix.

7. The steps in the method of making a metallic structure comprising: sintering together finely divided, non-compacted metal powders, to form porous metal matrix, impregnating the matrix formed with a mixture of metal including at least one metal which is readily alloyable with the metal of the matrix and another metal which is not readily alloyable with the metal of the matrix at a temperature only slightly above the

melting point of the impregnating alloy and for such a short time as to prevent any substantial dissolving action by the readily alloyable metal upon the matrix, then subsequently heating the impregnated porous metal matrix at a temperature well above the impregnating temperature and thereby causing the readily alloyable metal to diffuse into the metal of the matrix and form an alloy therewith without destroying the continuous structure of the matrix and leaving a distribution of the remainder of the mixture of the metal impregnant within the pores of the matrix.

ROLAND P. KOEHRING.

5

15